

# UNITED STATES PATENT OFFICE.

JOHN C. WOODRUFF, OF BAYONNE, NEW JERSEY, ASSIGNOR TO THE SOUTHERN COTTON OIL COMPANY, OF NEW YORK, N. Y., A CORPORATION OF NEW JERSEY.

## PREPARING NICKEL HYDROXID.

1,143,343.

Specification of Letters Patent. Patented June 15, 1915.

No Drawing.

Application filed January 29, 1913. Serial No. 744,837.

To all whom it may concern:

Be it known that I, JOHN C. WOODRUFF, a citizen of the United States, residing at Bayonne, Hudson county, New Jersey, have invented certain new and useful Improvements in Preparing Nickel Hydroxid, of which the following is the specification.

As is already known to the art, an efficient catalyst may be made by precipitating an oxy-hydrogen compound of nickel and applying the flocculent precipitate to the surface of an inert carrier or support, and thereafter heating the precipitate and the carrier to a temperature of about 500° C. in a current of hydrogen until the nickel has been reduced to a finely divided condition covering the support.

My invention relates to a method of precipitating hydroxid of nickel by use of an ammonium compound in such a manner that the precipitate will be relatively stable and the nickel will not form a soluble ammonium-nickel compound.

In carrying out my invention, nitrate of nickel or other nickel oxygen salt is dissolved in sufficient water to form a dilute solution, which should contain about 1% of the crystalline salt, and the solution is then brought to a temperature in the neighborhood of the boiling point. I have found that satisfactory results are obtained at a temperature of approximately 95° C. Sufficient hydroxid of ammonium to theoretically precipitate all the nickel present is then added. In practice I use an ammonium-hydroxid solution of a specific gravity of about 26° Baumé, but this is not an essential detail. The correct amount of a given solution of the ammonium hydroxid to add to the solution of the nickel salt may be determined by slowly adding the ammonium to a small quantity of the nickel solution under the above conditions, and noting the point at which the precipitate commences to dissolve. A slightly smaller proportion of the ammonium compound should then be

added to the bulk of the nickel solution. Under these conditions it will be found that practically all the nickel will be precipitated in the form of flocculent nickel hydroxid. 50 If a more concentrated nickel solution be employed or if precipitation be brought about at a lower temperature or if an excess of ammonia be added, the amount of nickel thrown down will be relatively decreased. 55

After the nickel hydroxid is precipitated it may be applied to the support while still in the solution in which it was formed, or the supernatant liquid may in the manner already known to the art be decanted off. 60 While this manner of applying the precipitate to the support is not part of my invention, I find that by the use of a very dilute solution of the nickel salt from which the precipitate is formed, practically all of 65 the impurities will be removed when the supernatant liquid is decanted off, whether before or after the application of the precipitate to the support, thus eliminating the necessity of washing the catalyst. The 70 precipitate and the support are then dried to expel water and are heated to a temperature of about 500° C. in a current of hydrogen.

The temperatures and strengths of solutions specified above are those at which I have obtained the best results, but I do not desire to limit myself to them, as the same results, to a certain extent, may be obtained when variations from the above are used. 75 80

I claim as my invention:

The method of precipitating nickel hydroxid, which consists in treating a solution of a nickel salt approximately 1% in strength at a temperature above 90° C. with 85 the theoretical amount of ammonium hydroxid necessary to precipitate the nickel present.

JOHN C. WOODRUFF.

Witnesses:

H. E. LONG,  
G. S. HANSEN.

Copies of this patent may be obtained for five cents each, by addressing the "Commissioner of Patents, Washington, D. C."